

## UNITED STATES PATENT OFFICE

2,087,766

## METHOD OF MAKING ROLLED PRODUCTS

Duncan P. Forbes, Erwin J. Mohr, and Fritz W. Meyer, Rockford, Ill., assignors to Gunite Foundries Corporation, Rockford, Ill., a corporation of Illinois

No Drawing. Application March 11, 1933,  
Serial No. 660,440

## 13 Claims. (Cl. 148—12)

This invention relates to the manufacture of rolled products of graphitic iron and we have successfully made rolled sheets, plates and bars of such metal by the methods herein set forth.

5 By the term graphitic iron we mean iron containing any form of precipitated free carbon, and by the term graphite we mean such free carbon.

The invention contemplates a generally improved and novel method for the manufacture of rolled shapes of graphitic iron wherein the cost of manufacture and the time required to carry out the method are materially reduced and wherein numerous difficulties incident to the 15 manufacture of such products are overcome.

The products are novel and commercially useful materials having among other properties advantageous corrosion resistant qualities. These products may be used for many purposes for 20 which steel sheets, plates and bars are ordinarily used and are preferable to steel for some purposes.

In our copending application, Serial No. 658,764, filed February 27, 1933, we have described a method for making rolled graphitic iron wherein white iron may be subjected to a heat treatment prior to rolling for the purpose of decomposing the cementite. While such treatment brings about favorable rolling conditions and permits greater reductions at each pass through the rolls, there are certain disadvantages to such a method. For example, when the composition of the metal is such that long heating periods are required to decompose the cementite, decarborization of the surface of the ingots may occur. Furthermore, it will be obvious that certain expense is involved in such heat treatment for fuel in heating the furnace and labor in transferring the ingots. Furthermore, 30 this heat treatment consumes a certain amount of time which in some instances would also be disadvantageous.

We have found through the actual manufacture of such products that certain advantages 45 will accrue from rolling the white iron ingots as such without prior heat treatment. We have found that by rolling the white iron directly, the rate of decomposition of the cementite may be accelerated and that the cementite will be largely 50 eliminated, and with metal of some analysis may be entirely eliminated, during the relatively short time required for rolling. In other words, the cementite decomposes at a much faster rate while the metal is being rolled than would otherwise be 55 the case at the same temperature. Consequently,

when the metal is rolled as ingots of white iron, the cementite will be entirely or largely eliminated during the rolling operations, thus either entirely obviating the necessity for heating the metal to decompose the cementite or greatly 5 reducing the time required to bring this about. Therefore, in most instances a great economy is effected by proceeding directly to the heat treating of metal to produce any of a plurality of matrices or complete the elimination of combined 10 carbon from the metal as hereinafter described, while the metal is still in the heat of rolling.

The first step in the method consists in the production of suitable ingots of white cast iron. The ingots may have any convenient size or shape 15 and may be formed by pouring into metal molds, green or dry sand molds, or core sand, or any other molds customary in foundry practice. The analysis of this iron will depend to some extent upon the heat treatment adopted and upon the 20 ultimate product desired, as will presently be described. The ingots will contain a certain proportion of massive cementite (iron carbide) which under heat treatment can be decomposed with a resultant precipitation of graphite in the 25 metal. Unless otherwise expressly stated the term cementite used throughout this specification and the appended claims is intended to mean iron carbide as a distinct crystalline constituent formed upon solidification of the metal and not 30 cementite formed at temperatures below this point. We heat these white iron ingots to a rolling temperature and while at this elevated temperature roll the ingots into the desired shapes, such as sheets, bars, and the like. 35

Our experience teaches us that in general the rolling can best be carried out at temperatures between about 1800° F., and the temperature at which a liquid phase begins to appear in the metal. In most cases this will be about 2100° F. 40 It may be possible, however, with metal of certain analysis to roll at slightly lower temperatures, but, in general, it seems that the best rolling temperature is the highest temperature obtainable without the presence of a liquid phase. 45 Any conventional rolling mechanism may be employed, but it will be found that as rolling proceeds, the operation becomes increasingly difficult. This we have found to be due to the rapid drop in temperature of the iron and the rapid decrease in ductility with change in temperature. However, if the metal is reheated one or more times during the rolling to maintain the temperature above about 1800° F., the desired reduction 50 in section may be satisfactorily accomplished. 55

It is, therefore, advisable to locate the heating furnace in such proximity to the rolling process as to prevent excessive loss in temperature of the metal between the heating furnace and the rolls. Care should be taken to select the proper amount of reduction at each pass. The amount of reduction at each pass will depend upon the temperature of the metal as it enters the rolls, the type of billet, the type of mill, the speed of rolling and also the intricacy of the shape being rolled, and other factors all of which are familiar to rolling mill operators who are experienced in handling metals which are rolled with difficulty.

We also contemplate heat treating the metal subsequent to the rolling operations to impart thereto certain commercially desirable characteristics, though for certain purposes the product of the rolling operations may be used directly without further treatment. This heat treatment contemplates various forms adapted to produce a product of commercially usable characteristics and involves the heat treatment of the metal, the type of heat treatment depending upon the ultimate product desired and the analysis of the metal. Thus, in order to produce a product of predetermined physical characteristics, we control both the analysis of the metal and the heat treatment imparted to the metal. This heat treatment also results in the production of uniform products from rolled materials which might otherwise have uncertain and erratic microstructure. The heat treatment thus serves two purposes, that of bringing the parts of each rolled form and also the various rolled forms to uniformity and that of imparting desired structural characteristics to the material.

One purpose of the present invention is to produce a rolled graphitic iron wherein the graphite is distributed in a matrix of ferrite. To produce such a material, we may take a rolled material, formed in the manner above described, from white iron ingots capable of being graphitized and having a carbon content preferably not less than 1.5%, a percentage of carbon plus a percentage of silicon greater than about 2.9%, and a manganese content which is twice the percentage of sulphur plus about .10% to .30%. When this iron is such that the percentage of carbon is about 1.5% to 2.20% and the percentage of carbon plus the percentage of silicon content is greater than 3.10%, preferably about 3.5%, the cementite of the metal will have been completely decomposed during the rolling operation, while with metal falling within substantially the remainder of the first above-mentioned range there is apt to be a certain amount of residual cementite after the rolling operations are completed. After the rolling operations, the rolled metal is placed in a furnace and is held within the graphitizing range (with most metals between 1350° F. and 1750° F.) until the cementite has been completely broken down. Where the metal is of an analysis such that the cementite is completely broken down during the rolling operations, this step may be eliminated. The metal is then cooled very slowly through the critical temperature until the combined carbon has been completely precipitated, or as an alternative the metal is held at a temperature which is below the critical temperature until the combined carbon has been decomposed to form graphite. The metal is then cooled to atmospheric temperature, preferably at a rapid rate. The resultant product will be material having the graphite in elongated sub-

stantially parallelly arranged form dispersed in a matrix of ferrite. Examples 1 and 2 are given by way of illustration, Example 1 illustrating the manner in which a material may be made wherein the cementite is completely decomposed during the rolling operations, while Example 2 illustrates the method wherein the metal as it comes from the rolls contains some residual cementite.

*Example 1.*—An ingot of  $\frac{3}{4}$ " thickness was prepared of white iron of the following analysis: Carbon 1.7%, silicon 1.65%, manganese .30%, sulphur .08%, phosphorous .10%. This ingot was heated to 1950° F., and as soon as it had reached a substantially uniform temperature was rolled into sheets of a thickness of  $\frac{1}{16}$  inch using a reduction of approximately 15% for each pass through the rolls. (We have used a 30% reduction at each pass with satisfactory results.) When the temperature of the metal dropped below about 1800° F., it was reheated to 1950° F. and rolling continued until the desired size and thickness of sheet was obtained, reheating as frequently as necessary to keep the material in rollable condition. After rolling was completed, the material was placed in a heat treating furnace before excessive loss of temperature had occurred and was held at about 1350° F. for twelve hours. It was then removed from the furnace and allowed to cool in air.

*Example 2.*—An ingot was prepared of white iron of the following analysis: Carbon 2.40%, silicon .90%, manganese .30%, sulphur .08%, and phosphorous .16%. These white iron ingots were heated to 1950° F. and rolled as soon as they had reached uniform temperature using a reduction of approximately 15% for each pass through the rolls. As described in Example 1, the metal was reheated as frequently as necessary to maintain it in condition. After rolling was completed, the material was placed in a heat treating furnace before excessive loss of temperature had occurred and held at about 1700° F. for eight hours. The metal was then cooled in the furnace to 1350° F. and held for twenty-four hours. Thereafter the rolled metal was removed from the furnace and allowed to cool in air.

In both Examples 1 and 2, the final product consisted of a rolled graphitic iron wherein the graphite or "temper carbon" was in the form of elongated substantially parallelly disposed deposits in a matrix of ferrite.

However, as previously pointed out, valuable products may be obtained without heat treating the metal after the rolling operations, though these products may lack uniformity in structure and physical properties unless operating conditions are carefully controlled.

*Example 3.*—White iron ingots having the analysis given in Example 1 were rolled as therein described and immediately after the rolling operations the rolled metal was cooled to atmospheric temperature. The resultant product consisted of a matrix which was largely pearlitic but contained a small amount of massive cementite and elongated parallel deposits of graphite.

*Example 4.*—White iron ingots having the analysis given in Example 2 were rolled as therein described and the rolled metal was allowed to cool to atmospheric temperature immediately after rolling. The product contained no massive cementite, and the matrix was largely pearlitic—having elongated substantially parallelly disposed deposits of graphite.

The invention also contemplates the production of rolled shapes wherein the matrix consists

of pearlite or sorbite. For the production of such a product, we prefer to start with a white iron which has a carbon content preferably not less than about 1.5%, a percentage of carbon plus a percentage of silicon content greater than about 2.9%, and a manganese content which is twice the percentage of sulphur plus .10% to .80% preferably twice the percentage of sulphur plus .30% to .80%. Higher manganese can be used but there appears to be no advantage in doing so. If the composition of the white iron is such that the carbon is between about 1.5% and 2.2%, and the percentage of carbon plus the percentage of silicon is greater than about 3.10%, preferably about 3.50%, the cementite will normally be completely decomposed during the rolling operations. These white iron ingots are rolled, as previously described, and then placed in a heat treating furnace. Where the analysis of the iron is such that there will be residual cementite in the metal after the completion of the rolling operations, the metal is held at a temperature within the graphitizing range until the cementite has been completely decomposed. The metal is then brought to above the critical temperature, but preferably not more than about 200° F. thereabove and is then cooled through the critical temperature at a speed such as to retain the combined carbon in the matrix in the form of pearlite or sorbite. The best results are usually obtained when cooling takes place rapidly in air. Examples 5 and 6 are given by way of illustration, Example 5 illustrating a method wherein the cementite is completely decomposed in the rolls, and Example 6 showing a method wherein the product of the rolling operations contains residual cementite.

*Example 5.*—A white iron ingot having a carbon content of 1.70%, silicon 1.65%, manganese .50%, sulphur .08%, and phosphorous .10% was heated to about 1950° F. and rolled as soon as the metal had become uniform in temperature, using a reduction of about 15% at each pass, the metal being reheated as frequently as necessary to maintain it in rolling condition. The metal was then placed in a heat treating furnace and brought to about 1600° F. only long enough to secure uniform temperature. Thereafter the metal was cooled rapidly to atmospheric temperature as by cooling in air.

*Example 6.*—A white iron ingot was made of the following analysis: Carbon 2.40%, silicon .90%, manganese .80%, sulphur .07%, and phosphorous .16%. The ingots were then heated to about 1950° F. and rolled as described in the first example as soon as it had become substantially uniform in temperature. The product of the rolling operation was then placed in a heat treating furnace and brought to about 1700° F. for eight hours, and was then brought to a uniform temperature of about 1600° F. and thereafter cooled rapidly through the critical temperature to room temperature, for example, as by cooling in air.

The products of the methods described in Examples 5 and 6 showed a pearlitic matrix containing elongated clusters of graphite or temper carbon.

The invention also contemplates the production of products wherein the matrix consists of spheroidized eutectoid cementite distributed through ferrite crystals. In making such a product, we prefer to roll a white iron ingot wherein the carbon is preferably not less than about 1.5%, the percentage of carbon plus the percentage of silicon is greater than about 2.9%, and the man-

ganese content is about twice the percentage of sulphur plus .10% to .80%, preferably twice the percentage of sulphur plus .30% to .80%. The ingots are heated directly to the rolling temperature and rolled, as previously described. The product of the rolling operations is placed in a furnace and held within the graphitizing range until the residual cementite has been completely decomposed. The metal is then cooled through the critical temperature at a speed such as to retain the combined carbon in the matrix in the form of pearlite or sorbite, as for example by cooling in air, and is then held at or reheated to the spheroidizing range (about 1200° F. to 1300° F.) for a sufficient time to spheroidize the pearlite or sorbite to the desired degree. Example 7 is given by way of illustration of a satisfactory manner of producing this type of product.

*Example 7.*—A white iron ingot having the analysis set forth in Example 5 was made and rolled in the manner already described. After the material had been rolled to the desired shape it was held at about 1700° F. for about eight hours and was then cooled at the rate of about 600° per hour through the critical temperature (in this case about 1375° F.) and then held at a temperature of about 1275° F. for twenty-four hours. It was thereafter cooled to room temperature. This metal had a matrix of finely spheroidized cementite uniformly distributed through ferrite crystals and elongated substantially parallel disposed deposits of graphite were embedded in this matrix.

It will be seen that in our process we use as a starting point white iron and proceed to roll this metal at an elevated temperature. In this way, we are enabled to materially accelerate the rate at which the cementite is decomposed, thereby materially reducing the time required for the production of certain desirable products. By properly regulating the analysis of the metal, we are enabled to bring about complete decomposition of the cementite during the rolling operations, thereby completely eliminating the necessity for holding the metal at an elevated temperature until the cementite has been decomposed. In those instances where the cementite is not completely decomposed during the rolling of the metal, the heat treatment required for the completion of this decomposition is greatly reduced in time and may be combined with some other subsequent heat treatment and be carried out in the same furnace, as a preliminary step of such heat treatment. In this manner, frequent transfers of the metal from furnace to furnace is eliminated and a considerable saving in heat and time is effected since what would otherwise be two separate heat treatments are combined into a single continuous treatment at required temperatures.

The amount of the decomposition of the cementite will depend to a certain degree upon the extent of the working of the metal but in commercial operations the reduction of section is usually sufficient to result in the decomposition of at least a large part of the cementite and when the analysis is favorable, as herein described, all of the cementite will be decomposed. Some allowances will have to be made when the rolling operations depart from the customary reductions.

As one phase of our invention, we regulate the analysis of the white iron, and, after rolling, subject the rolled material to certain heat treatments to produce uniform products of definite,

yet variable physical properties. This heat treatment normally serves two purposes. It serves first to produce resultant products of certain predetermined physical properties, thereby enabling us to produce products suitable and valuable for certain definite requirements. However, in addition to this function of the heat treatment, the steps also serve to bring the rolled metal into uniformity regardless of the particular nature of its matrix. It will be understood that during and prior to the rolling operations the ingots are subjected to variable conditions so that in many instances there will be a variation in the microstructure of the metal of the different ingots, and frequently a variation in the microstructure of various parts of the same sheet or bar rolled from an ingot. For some uses the metal will, of course, be satisfactory regardless of these variables. However, the heat treatment after the rolling operations serves to overcome this lack of uniformity so that the product of the method may have uniformity throughout each piece and throughout the various pieces.

New and novel products result from the method above disclosed, such products being described and claimed in our above-mentioned copending application. These products have certain new and commercially valuable properties. Cast iron and metals containing graphite have long been well known for their corrosion resistance properties, particularly corrosion due to atmospheric exposure and underground services. For this use the metals must in many cases be thin in section. In the past, metals for this purpose have been non-ferrous metals or steel alloys which contain substantial quantities of other metals, such as chromium, copper, nickel, etc. These alloys are relatively expensive. The difficulty has been that while iron containing graphite has in the past been available in the form of individually cast plates, there is a limitation to the minimum section which can be cast of graphite bearing iron. That is, in the past there has been no method of making graphite bearing iron in sheets of sufficient size and thinness of section to permit the general use of such metals for corrosion resistance purposes or for other purposes to which such metal in the sheet form might be adapted. Our method completely obviates this difficulty and permits the rolling of such metal in very thin section and in relatively large sheets. The method brings about the production of uniform sheets of graphite bearing metal of predetermined properties with almost the same facility with which steel sheets are made, thus opening up a large variety of new materials for the sheet metal industry. The method also permits the production of graphite bearing metal in shapes and sizes which have heretofore not been obtainable.

A number of uses for the metals made in accordance with our method might be listed. The metal made in accordance with Examples 1 and 2 is valuable for use in fabrication where drawing and forming operations are necessary. The metal made in accordance with Examples 5 and 6 will be of particular value where wear resistance and corrosion resistance are important, such, for example, as in the manufacture of elevator buckets. Metal made in accordance with the seventh example possesses corrosion resistance as well as high strength and ductility, and is of particular value in the manufacture of such materials as ship plates, coal hoppers, tanks, and the like.

We have dealt throughout this specification with the composition of the metal as this is concerned with certain well known constituents. It will be understood, however, that numerous other elements may be present in the metal or may be added thereto which will or may effect the method or the product—some beneficially and some otherwise.

While we have thus described and illustrated specific embodiments of our invention, we are aware that numerous alterations and changes may be made without departing from the spirit of the invention and the scope of the appended claims, in which—

We claim:

1. The method for treating graphitizable white cast iron containing a graphitizing agent to accelerate the decomposition of the cementite which includes heating said iron to a temperature above about 1800° F. and thereafter plastically deforming the same.

2. The method of rolling sheets, bars, and other shapes from graphitizable white cast iron containing a graphitizing agent wherein the decomposition of the cementite of the iron is accelerated by hot rolling of the metal above about 1800° F. and the metal is thereafter held at a temperature within the graphitizing range to decompose the residual cementite.

3. The method of making rolled shapes of graphitic iron, comprising bringing to the hot rolling temperature white iron wherein the carbon is about 1.5% to about 2.0% and the percentage of carbon plus the percentage of silicon is not less than about 3.10%, hot rolling said iron to deform the same and decompose the cementite, thereafter holding the rolled metal at a temperature in the region of the critical temperature until the combined carbon thereof has been substantially completely precipitated as graphite.

4. The method of making rolled shapes of graphitic iron, comprising bringing to a hot rolling temperature above about 1800° F. white iron of an analysis within the following limits—carbon not less than 1.5%, percentage of carbon plus percentage of silicon greater than about 2.9%, manganese equal to twice the percentage of sulphur plus .10% to .80%, rolling said iron, heat treating the same in the graphitizing range to decompose the cementite remaining after the rolling operations and cooling at a rate to produce a pearlitic matrix.

5. The method of making rolled shapes of graphitic iron, comprising bringing to the hot rolling temperature above about 1800° F. white iron wherein the carbon content is between about 1.5% and 2.20% and the percentage of carbon plus the percentage of silicon is not less than about 3.10%, rolling said iron and cooling said iron from a point slightly above the critical temperature at a speed such as to retain the combined carbon in the matrix in the form of pearlite.

6. The method of making rolled shapes of graphitic iron comprising bringing to the hot rolling temperature above about 1800° F. white iron of an analysis within the following limits—carbon not less than about 1.5%, percentage of carbon plus percentage of silicon greater than about 2.9%, manganese equal to twice the percentage of sulphur plus .10% to .80%, rolling said iron to deform the same and decompose the major portion of the cementite thereof, thereafter holding the same at a temperature within the graphitizing range to decompose the residual cementite, cooling the iron from a point slightly above the

critical temperature through the critical temperature at a speed such as to retain the combined carbon in the matrix in the form of pearlite, and then holding the metal at a spheroidizing temperature to spheroidize the pearlite.

7. The method of making rolled shapes of graphitic iron which consists in producing ingots of white cast iron containing a graphitizing agent, causing said ingots to be brought as ingots of white cast iron to a temperature above about 1800° F. but below the temperature at which a liquid phase appears in the metal of said ingots, and reducing said ingots to rolled forms of a desired size by rolling the ingots first while at substantially said high temperature and then successively while the ingots are at a temperature above about 1800° F., reheating of the ingots between successive rolling operations being resorted to when necessary to maintain the ingots at a temperature above about 1800° F. until so reduced.

8. The method for making rolled shapes of graphitic iron wherein white iron containing a graphitizing agent is rolled at temperatures above about 1800° F.

9. The method for making rolled shapes of graphitic iron wherein iron containing a graphitizing agent is rolled as ingots of white iron at a temperature above about 1800° F., and the rolled metal is then held at a temperature in the graphitizing range until the massive cementite is substantially completely decomposed.

10. The method of making rolled shapes of graphitic iron comprising bringing to a hot rolling temperature above about 1800° F. an iron carbon alloy of an analysis within the following

limits—carbon not less than about 1.5%, percentage of carbon plus percentage of silicon greater than about 2.9%, manganese equal to twice the percentage of sulphur plus about .10% to .30%, hot rolling said metal at a temperature above about 1800° F. and thereafter subjecting the rolled metal to a heat treatment in the graphitizing range to precipitate at least a portion of the combined carbon as graphite.

11. The method of making rolled shapes of graphitic iron, comprising bringing to the hot rolling temperature above about 1800° F. an iron carbon alloy wherein the carbon is about 1.5% to about 2.2% and the percentage of carbon plus the percentage of silicon is not less than about 3.10%, and hot rolling said metal to deform the same and decompose the cementite.

12. The method for making rolled shapes of graphitic iron wherein iron containing a graphitizing agent is rolled as ingots of white iron at temperatures above about 1800° F., the rolled metal is then held at a temperature in the graphitizing range until the cementite is substantially completely decomposed and is then subjected to a heat treatment to develop a predetermined microstructure of the matrix.

13. The method for making rolled shapes of graphitic iron wherein iron containing a graphitizing agent is rolled as ingots of white iron at temperatures above about 1800° F. to deform the same and decompose the cementite, and is thereafter subjected to a heat treatment to develop a predetermined microstructure of the matrix.

DUNCAN P. FORBES.

ERWIN J. MOHR.

FRITZ W. MEYER.

35

39